

Nov. 12, 1963

R. W. WOLLENTIN

3,110,837

ELECTROLUMINESCENT DEVICE AND METHOD

Filed April 4, 1961

FIG. 1.



FIG. 2.



FORM SOLVENT SOLUTION OF CANADA  
BALSAM AND ETHYLCELLULOSE.

APPLY SOLVENT SOLUTION AS A COATING  
TO METALLIC ELECTRODE FOR EL DEVICE.

MAINTAIN COATING AT ROOM TEMP. FOR AT  
LEAST 10 MINUTES.

HEAT COATING TO FROM 80° C. TO 110° C  
FOR FROM 5 TO 20 MINUTES.

MAINTAIN COATING AT ROOM TEMP. FOR  
AT LEAST 8 HOURS TO COMPLETELY DRY SAME.

APPLY MOISTURE- IMPERVIOUS LAYER OVER  
ALL MOISTURE - PERVERSUS PORTIONS OF  
EL DEVICE AND OVER DRIED COATING.

FIG. 3.

INVENTOR.

ROBERT W. WOLLENTIN.

BY

*W. D. Palmer*  
ATTORNEY.

# United States Patent Office

**3,110,837**

Patented Nov. 12, 1963

1

3.110.837

**3,110,637**  
**ELECTROLUMINESCENT DEVICE AND**  
**METHOD**

Robert W. Wollentin, Bloomfield, N.J., assignor to Westinghouse Electric Corporation, East Pittsburgh, Pa., a corporation of Pennsylvania

Filed Apr. 4, 1961, Ser. No. 100,701  
8 Claims. (Cl. 313—108)

This invention relates to electroluminescent devices and, more particularly, to an electroluminescent device which has improved operating characteristics and a method for making such an improved electroluminescent device.

The phenomenon of electroluminescence was first disclosed by G. Destriau, one of his earlier publications appearing in London, Edinburgh and Dublin Philosophical Magazine, Series 7, Volume 38, No. 285, pages 700-737 (October 1947). Since this time, considerable research and engineering effort has been expended on the phenomenon of electroluminescence and such devices have been marketed commercially. One of the main limitations to commercial utilization of electroluminescent devices is the inherent decrease in light output during operating life. The rate of light output decrease is known to be accelerated by the presence of moisture.

In order to prevent electroluminescent devices from being damaged by moisture, it has been suggested to encapsulate the moisture-pervious surface portions of such devices with a substantially moisture-impermeable material. Such encapsulating moisture-impermeable materials are normally fairly rigid, however, and if an incipient electrical breakdown occurs between the device electrodes, the resulting gases which are generated tend to cause the breakdown to become progressive in nature, thereby leading to the destruction of the electroluminescent layer. In addition, the encapsulating, substantially moisture-impermeable materials are often not completely effective in preventing ingress of moisture with the result that under high-humidity conditions of operation, the useful operating life of such electroluminescent devices is severely limited.

It is the general object of the present invention to avoid and overcome the foregoing and other difficulties of and objections to prior-art practices by the provision of an electroluminescent device which has improved life when operated under conditions of high humidity.

It is another object to provide an electroluminescent device having good maintenance of initial brightness and which device has protection against progressive arcing between the device electrodes after an incipient arc has occurred therebetween.

It is a further object to provide a method for making an improved electroluminescent device which has good maintenance of light output when operated in moist atmospheres and which device is protected against progressive arcing between electrodes.

The aforesaid objects of the invention, and other objects which will become apparent as the description proceeds, are achieved by providing an electroluminescent device wherein a prime coat layer consisting essentially of a mixture of from 80% to 50% by weight of Canada balsam and from 20% to 50% by weight of ethylcellulose having an ethoxyl content of from 47.5% to 49.0% is provided over one of the device electrodes. Over this so-called prime coat and over all moisture-pervious operative portions of the electroluminescent device is placed a layer of substantially moisture-impervious material, such as a layer of epoxy resin. The improved prime coat provides better protection against the deleterious effects of moisture and, in addition, tends to quench or suppress

2

incipient arcs which may occur between the device electrodes, in order to prevent such incipient arcs from becoming progressive in nature and destroying the device.

For a better understanding of the invention, reference should be had to the accompanying drawings wherein:

- 5 should be had to the accompanying drawings wherein:  
FIG. 1 is a sectional elevational view of an electro-  
luminescent device wherein the phosphor material is em-  
bedded in plastic dielectric and wherein the uppermost  
electrode is covered with the so-called prime coat of the  
10 present invention, with this prime coat and all moisture-  
permeable surface portions of the device being encased by  
a layer of substantially moisture-impervious material;  
FIG. 2 is a sectional elevational view of an alternative  
15 construction for a device embodiment generally as shown  
in FIG. 1, wherein an additional layer of material having  
high electrical puncture strength is also included between  
the device electrodes;  
FIG. 3 is a flow chart setting forth the steps of the  
20 present method.  
With specific reference to the form of the invention  
illustrated in the drawings, the numeral 10 in FIG. 1  
indicates generally an electroluminescent device comprising  
a first electrode 12 formed on a glass foundation 14.  
25 A layer 16 comprising electroluminescent phosphor em-  
bedded in light-transmitting dielectric material is positioned  
over the electrode 12 and a second conducting  
electrode layer 18 is positioned over the phosphor-di-  
electric layer 16. The spaced electrodes 12 and 18 and  
30 phosphor-dielectric layer 16 form the operative portion  
of the device 10. Over the second or uppermost elec-  
trode 18 and exterior to the operative portion of the  
device 10 is carried a prime coat 20 which is formulated  
35 in accordance with the present invention, as will be con-  
sidered in greater detail hereinafter. This prime coat  
has a thickness of at least 5 mils and preferably has a  
thickness of from 7 to 10 mils. Over the prime coat 20  
and also over all moisture-permeable portions of the de-  
30 vice 10 is carried an additional layer 22 of substantially  
moisture-impervious material which extends down onto  
the sides 24 of the foundation 14. Light which is gen-  
erated by the device 10 is emitted from the viewing face  
26 of the glass foundation 14. Energization of the device  
40 10 is effected through lead conductors 28 sealed through  
the moisture-impervious layer 22. These lead conductors  
are electrically connected to conventional bus bars 30,  
45 which in turn complete electrical contact to the device  
electrodes 12 and 18.  
The glass foundation 14 can be fabricated of any con-  
50 ventional light-transmitting glass material and as an ex-  
ample, the foundation 14 has a thickness of one-eighth  
inch. The first electrode 12 can be formed of a very thin  
coating of electrically conducting and light-transmitting  
tin oxide, and such electrode coatings are well known.  
55 Other similar coatings such as indium oxide can be sub-  
stituted therefor. The layer 16 comprising the phosphor-  
dielectric can be formed of any electroluminescent phos-  
phor embedded in light-transmitting dielectric material,  
with plastic dielectric being preferred for best brightness.  
60 As an example, the electroluminescent phosphor is formed  
of finely divided zinc sulfide which is activated by copper  
and coactivated by chlorine. Such phosphor is well  
known and other known electroluminescent phosphors  
are summarized in Destriau and Ivey article in "Proceed-  
65 ings of the I.R.E." Volume 43, No. 12, pages 1911-  
1940 (December 1955). For best initial brightness, the  
dielectric material in which the phosphor is embedded is  
preferably plastic and, as one example, a suitable plastic  
dielectric is polyvinyl chloride acetate. Other known  
70 plastic dielectric material can be substituted therefor. The  
relative proportions of phosphor and dielectric which  
comprise the layer 16 are not critical and by way of ex-

ample, two parts by weight of phosphor per one part by weight of dielectric are used in the layer 16. The thickness of the layer 16 is two mils and this thickness can be varied.

The second electrode 18 is formed of vacuum-metallized material, preferably aluminum, although other metals such as silver can be used. The thickness of the electrode 18 is not critical and as an example is 1500 A.U. The second electrode 18 need not be vacuum metallized and can be fabricated of a preformed sheet of aluminum or other metal, if desired. A vacuum-metallized electrode layer contains a plurality of voids which will permit ingress of liquid. This in turn can damage the device. The prime coat 20 of the present invention is particularly adapted for use with such a vacuum-metallized electrode layer, inasmuch as this prime coat prevents liquid from penetrating into such voids in the electrode layer.

The so-called prime coat 20 of the present invention is formed of a mixture of from 80% to 50% by weight of Canada balsam and from 20% to 50% by weight of ethylcellulose having an ethoxyl content of from 47.5% to 49.0%. The substantially moisture-impervious layer 22 is preferably formed of a material which at least principally comprises epoxy resin. Such epoxy resins represent a class of condensation polymers, are well known, and are available from a number of different manufacturers. A catalyst is normally used to promote polymerization of the resin. On polymerization the molecular chain lengthens and considerable cross-linking occurs between individual molecular chains. There are numerous suitable catalysts which can be used in forming the epoxy resin layer 22 and the preferred catalyst is a mixture of 50% by weight diethylene triamine and 50% by weight acrylonitrile. Many other suitable catalysts for these epoxy resins are known and for a further discussion of such resins, see "Epoxy Resins" by Lee and Neville, published by McGraw-Hill (1957). Other materials can be added to the epoxy resins in forming the layer 22 to modify the characteristics of this layer. As an example, from 20 to 45% by weight of a polyamide can be added to the epoxy resins to increase their flexibility. This inhibits any tendency for stress failure of the layer 22.

In fabricating the device 10, the phosphor-dielectric layer 16 is first applied to the light-transmitting electrode 12 by conventional practices and the second electrode 18 vacuum metallized onto the layer 16. As shown in the flow chart of FIG. 3, before applying the prime coat 20 to the exposed surface of the second electrode 18, Canada balsam and the indicated ethylcellulose are mixed together with a suitable solvent to a viscosity which will facilitate spraying. The preferred relative proportions by weight of Canada balsam to ethylcellulose are 60-40 and this preferred ratio will be considered in detail. As a specific example 150 grams of Canada balsam and 50 cc. of turpentine are mixed with 100 grams of ethylcellulose having an ethoxyl content of from 47.5% to 49.0%, known in the art as "N-type" ethylcellulose. To the mixed Canada balsam and ethylcellulose are added 400 cc. of toluene and 200 cc. of n-butyl acetate. The resulting mixture is diluted with toluene in the proportion of one part by volume of toluene to four parts by volume of the mix for spray application. The solvent solution is then applied as a coating to the exposed surface of the second conducting layer 18 in such amount that the solids component of the applied solution will dry to a total thickness of at least 5 mils and preferably from 7 to 10 mils. It is preferred to form the prime coat by applying successive layers, allowing for a short drying period between each applied layer. As an example, in forming an eight-mil-thick prime coat 20, this coating can be sprayed on as four successive layers, one on top of the other, each having a thickness of two mils. Thereafter the applied solvent-containing layer is maintained at room temperature for a period of at least ten minutes, and preferably for about fifteen minutes, in order to permit an appreciable

portion of the solvent therein to volatilize. Most of the remaining solvent is then volatilized from the applied coating by heating the coating at a temperature of from 80° C. to 110° C. for a period of from five minutes to twenty minutes, with the higher the heating temperature, the shorter the heating time. Preferably the coating 20 is heated to a temperature of about 100° C. for a period of from seven to ten minutes. Thereafter the applied coating 20 is maintained at room temperature for an additional period of at least 8 hours, in order to permit any residual solvent therein to volatilize therefrom.

The initial solvent coating drying period of at least ten minutes at room temperature has been found necessary to permit an appreciable portion of the solvent in the applied coating to volatilize at a relatively slow rate. If the coating were immediately heated after application in order to volatilize solvent, there would be some tendency to develop a "skin" over the applied coating. The follow-up heating period, as indicated, serves to drive nearly all remaining solvent from the applied coating. It has been found that any residual solvent remaining in the applied coating will damage the performance of the electro-luminescent device. The last prolonged holding period at room temperature, as indicated hereinbefore, serves to permit any residual solvent to volatilize from the applied coating before the device is encapsulated, in order to insure that the performance of the device is not impaired by any entrapped residual solvent.

The partially fabricated device is then either dipped 30 into an unpolymerized epoxy resin-catalyst mixture or such epoxy resin mix is flowed thereover to cover the applied layer 20 and moisture-permeable surface portions of the device 10. In the case of the preferred indicated catalyst, resin polymerization is accomplished by heating 35 the resin-coated device to a temperature of 50° C. for thirty minutes. In the device embodiment 10, as shown in FIG. 1, the epoxy resin layer 22 covers the back portion of the device including the prime coat 20 and extends down onto the sides of the device so as to form a substantially 40 moisture-impervious seal with the sides 24 of the glass foundation 14. As an example, the epoxy resin layer 22 has a thickness of 45 mils. This thickness is not critical and is subject to considerable variation.

In FIG. 2 is shown a further device embodiment 10a which generally corresponds to the embodiment 10, as shown in FIG. 1, except that an additional layer 32 of material having a very high electrical breakdown resistance is also included between the device electrodes 12 and 18. Such an additional layer can be formed of barium titanate or titania for example, as disclosed in British Patent No. 765,076, published October 22, 1954. The device embodiment 10a, as shown in FIG. 2 is also modified somewhat in that the layer 22a, which comprises light-transmitting epoxy resin, encapsulates the entire device. Such a construction lends itself to a dip process for applying the epoxy resin layer 22a.

In controlled tests, electroluminescent devices incorporating the improved prime coat of this invention were operated at a temperature of 50° C. and at a relative humidity of approximately 98%. The control electroluminescent devices were otherwise similar but incorporated, as a so-called prime coat, an equivalent layer of Canada balsam which was not modified by the addition of the specified ethylcellulose. The devices incorporating the improved prime coat of the present invention 60 operated for approximately twice as long as the control devices before the first indication of deleterious moisture penetration. Also, under normal ambient operating conditions, the devices incorporating the present improved prime coat operated for approximately twice as long as 65 the control devices before the light output dropped to one-half of its initial value. In addition, when incipient arcs did occur, both the control devices and the present devices acted to quench the arcs and prevent them from 70 becoming progressive.

75 Devices incorporating a prime coating formed of Can-

ada balsam, without the addition of ethylcellulose in accordance with the present invention, are limited in operating temperature because of the low melting point of Canada balsam, which is about 80° C. In addition, the Canada balsam is a relatively expensive material to purchase. A mixture of 60% by weight Canada balsam and 40% by weight ethylcellulose has a melting point of about 105° C. so that the temperature range under which the device can be operated is appreciably increased when the present improved prime coat is used.

If less than 20% by weight of the specified ethylcellulose is utilized, the melting point for the prime coat layer 20 will be decreased to about 90° C. or less. From a commercial standpoint, this is barely acceptable. If more than 50% by weight of the specified ethylcellulose is utilized, the melting point of the prime coat layer 20 increases further, but the coating layer is overly hard and brittle. As a result, there is lack of adherence of the prime coat layer to the operative portion of the device. In addition, because of the increased melting point and brittleness, the arc-suppressant qualities of such a coating layer are impaired, apparently because the coating layer does not melt rapidly enough to enable the gases generated on incipient breakdown to be dissipated in sufficiently rapid fashion to quench such an incipient arc. If the coating layer 20 is less than 5 mils in thickness, the performance of the device is somewhat marginal from the standpoint of protecting the device from progressive arcing and possible contamination by the overlying layer of substantially moisture-impermeable material. As indicated hereinbefore, the preferred thickness for the layer 20 is from 7 to 10 mils. There appears to be no technical limitation to how thick the layer 20 can be, except as limited by the considerations of cost of materials and cost of manufacture.

Other materials can be utilized to replace the epoxy resin in forming the moisture-impermeable layer 22. As an example, the layer 22 can be formed of glass which is adhered to the prime coat layer 20 by means of a very thin layer of epoxy resin.

As a possible alternative embodiment, the plastic dielectric material which is used as an embedding medium for the phosphor can be replaced by a glass or ceramic dielectric, such a construction being well known. In accordance with the present invention, the prime coat still would be placed over the uppermost electrode and the entire device encapsulated with the substantially moisture-impermeable material, in order to inhibit any ingress of moisture to the operative portions of such a ceramic-type device.

It will be recognized that the objects of the invention have been achieved by providing an electroluminescent device which operates very well under conditions of high humidity as well as in a normal environment. In addition, this device is not subject to progressive arcing between the electrodes. There has also been provided a method for fabricating such an improved device.

While best embodiments of the invention have been illustrated and described in detail, it is to be particularly understood that the invention is not limited thereto or thereby.

I claim:

1. An electroluminescent device comprising, a light-transmitting first electrically conducting layer carried on a light-transmitting foundation, a second electrically conducting layer spaced from said first conducting layer, a layer comprising electroluminescent phosphor included between said first and said second conducting layers, said first and said second conducting layers and said layer comprising electroluminescent phosphor defining the operative portion of said device, a prime coat having a thickness of at least 5 mils carried on said second conducting layer and external to the operative portion of said device, said prime coat consisting essentially of a mixture of from 80% to 50% by weight of Canada

balsam and from 20% to 50% by weight of ethylcellulose having an ethoxyl content of from 47.5% to 49.0% and a substantially moisture-impermeable layer over said prime coat and encapsulating all moisture-permeable operative portions of said device.

5 2. An electroluminescent device as specified in claim 1, wherein said substantially moisture-impermeable layer at least principally comprises epoxy resin.

10 3. An electroluminescent device as specified in claim 1, wherein said second conducting layer contains a plurality of voids which will permit ingress of liquid.

15 4. An electroluminescent device comprising, a light-transmitting first electrically conducting layer carried on a light-transmitting foundation, a second electrically

conducting layer spaced from said first conducting layer, a layer comprising electroluminescent phosphor included between said first and said second conducting layers, said first and said second conducting layers and said layer comprising electroluminescent phosphor defining the operative

20 portion of said device, a prime coat having a thickness of from 7 to 10 mils carried on said second conducting layer and external to the operative portion of said device, said prime coat consisting essentially of a mixture of about 60% by weight of Canada balsam and about 40% by

25 weight of ethylcellulose having an ethoxyl content of from 47.5% to 49.0% and a substantially moisture-impermeable layer over said prime coat and encapsulating all moisture-permeable operative portions of said device.

5 5. The method of protecting from damage by moisture

30 an electroluminescent device comprising a light-transmitting first electrically conducting layer carried on a light-transmitting foundation, a second electrically conducting layer spaced from said first conducting layer, and a layer comprising electroluminescent phosphor included between

35 said first and said second conducting layers, which method comprises: forming a solvent solution having dissolved solids consisting essentially of from 80% to 50% by weight Canada balsam and from 20% to 50% by weight ethylcellulose having an ethoxyl content of from

40 47.5% to 49.0%; applying said solvent solution as a coating to the exposed surface of said second conducting layer in such total thickness that the solids components of such applied solvent coating will dry to a thickness of at least 5 mils; maintaining said applied solvent coating

45 at room temperature for a period of at least ten minutes to permit an appreciable portion of solvent therein to volatilize therefrom; further volatilizing solvent from the applied coating by heating same at a temperature of from 80° C. to 110° C. for a period of from five minutes to twenty minutes, with the higher the heating temper-

50 ature the shorter the heating time; maintaining said applied coating at room temperature for an additional period of at least eight hours to permit any residual solvent therein to volatilize therefrom; and thereafter applying

55 a substantially moisture-impermeable layer over said applied Canada balsam-ethylcellulose coating as well as over all moisture-permeable portions of said device.

6. The method as specified in claim 5, wherein said solvent solution is initially applied as a plurality of suc-

60 cessive coatings to the exposed surface of said second conducting layer, with the total thickness of such applied coatings being such that the solids components thereof will dry to a thickness of at least 5 mils.

7. The method as specified in claim 5, wherein said solvent solution is applied as a coating to the exposed surface of said second conducting layer in such total thickness that the solids components of such applied solvent coating will dry to a thickness of from 7 mils to 10 mils.

70 8. The method of protecting from damage by moisture an electroluminescent device comprising a light-transmitting first electrically conducting layer carried on a light-transmitting foundation, a second electrically conducting layer spaced from said first conducting layer, and a layer comprising electroluminescent phosphor including be-

tween said first and said second conducting layers, which method comprises: forming a solvent solution having dissolved solids consisting essentially of from 80% to 50% by weight Canada balsam and from 20% to 50% by weight ethylcellulose; applying said solvent solution as a coating to the exposed surface of said second conducting layer in such total thickness that the solids components of such applied solvent coating will dry to a thickness of from 7 to 10 mils; maintaining said applied solvent coating at room temperature for a period of about fifteen minutes to permit an appreciable portion of solvent therein to volatilize therefrom; further volatilizing solvent

5  
10

from the applied coating by heating same at a temperature of about 100° C. for a period of from seven minutes to ten minutes; maintaining said applied coating at room temperature for an additional period of at least eight hours to permit any residual solvent therein to volatilize therefrom; and thereafter applying a substantially moisture-impervious layer at least principally comprising epoxy resin over said applied Canada balsam-ethylcellulose coating as well as over all moisture-pervious portions of said device.

No references cited.